

# United States Patent

Iwano et al.

[15] 3,649,281

[45] Mar. 14, 1972

[54] **PHOTOGRAPHIC PROCESSING FOR  
PHOTOGRAPHIC SILVER HALIDE  
LIGHT-SENSITIVE ELEMENTS**

[72] Inventors: **Haruhiko Iwano; Isao Shimamura**, both of Kanagawa, Japan

[73] Assignee: **Fuji Photo Film Co., Ltd.**, Kanagawa, Japan

[22] Filed: **Oct. 4, 1968**

[21] Appl. No.: **765,032**

[30] **Foreign Application Priority Data**

Oct. 4, 1967 Japan.....42/63936

[52] U.S. Cl. .... **96/66.5, 96/50 PT, 96/109,  
96/111**

[51] Int. Cl. .... **G03c 5/30**

[58] Field of Search ..... **96/66.5, 109, 22, 50, 50 PT,  
96/111; 260/621, 623, 625, 456, 473, 512, 521,  
556, 559, 613**

[56] **References Cited**

UNITED STATES PATENTS

2,165,421 7/1939 Sheppard et al. ....96/111  
2,586,168 2/1952 Kaszuba.....96/109 X

FOREIGN PATENTS OR APPLICATIONS

504,378 4/1939 Great Britain .....96/109

Primary Examiner—William D. Martin

Assistant Examiner—M. R. Lusignan

Attorney—Sughrue, Rothwell, Mion, Zinn & Macpeak

[57] **ABSTRACT**

In photographic processings for photographic silver halide light-sensitive elements which include a prehardening step and development step, an improvement which comprises processing the light-sensitive element between the prehardening step and the development step in an aqueous solution containing a resorcinol derivative represented by the following general formula:



The moieties A and B are defined in the specification.

4 Claims, No Drawings

## PHOTOGRAPHIC PROCESSING FOR PHOTOGRAPHIC SILVER HALIDE LIGHT-SENSITIVE ELEMENTS

## BACKGROUND OF THE INVENTION

## 1. Field of the Invention

The present invention relates generally to photographic processing for photographic silver halide light-sensitive elements, and more particularly to a process for reducing the formation of fog occurring during hardening silver halide emulsion layers.

## 2. Description of the Prior Art

In general, when photographic light-sensitive films, photographic printing papers or photographic light-sensitive plates having silver halides are processed after exposure, they are frequently subjected to hardening processing prior to development.

The object of the hardening process is to prevent emulsion layers from being mechanically damaged during processing by increasing the mechanical strength of the emulsion layers of photographic silver halide light-sensitive elements, and in particular, the application of the hardening processing is quite effective when the mechanical strength of the photographic emulsion layers is originally insufficient, the photographic emulsion layers are processed for a long period of time, or they are processed in a processing solution having a high pH or a high temperature.

The hardening processing conducted before the development step is usually called "prehardening," and as a hardening agent for the processing, there is usually employed an aldehyde capable of hardening gelatin in the photographic emulsion layer by reaction therewith, such as formaldehyde, glyoxal, succinaldehyde, glutaraldehyde, and the like.

Although the photographic emulsion layers are effectively hardened by this kind of prehardening processing, it has a bad influence on the photographic properties of the photographic emulsion layers thus processed, for example, the formation of development fog is increased, the development density at reversal development is reduced, and the coupling property of couplers in photographic light-sensitive color elements is varied.

## SUMMARY OF THE INVENTION

It has been discovered that in photographic processes of photographic silver halide light-sensitive elements wherein the processes include a prehardening step and a development step, it has been discovered that improved mechanical strength, lowered formation of development fog, lowered development density at reversal development, and better coupling properties are obtained by processing the light-sensitive element between the above-mentioned prehardening step and the development step in an aqueous solution containing a resorcinol derivative represented by the following general formula:



A and B each represent a member selected from the group consisting of a hydrogen atom, a lower alkyl group, a halogen atom, OR<sub>1</sub> (wherein R<sub>1</sub> is a lower alkyl group), ZOR<sub>2</sub> (wherein R<sub>2</sub> is a member selected from the group consisting of a hydroxyl group, an alkoxyl group, and NH<sub>2</sub>), and SO<sub>2</sub>R<sub>3</sub> (wherein R<sub>3</sub> is a member selected from the group consisting of a hydroxyl group, an alkoxyl group, and NH<sub>2</sub>).

Therefore, an object of the present invention is to provide an improved photographic processing for photographic light-sensitive elements capable of providing sufficient mechanical strength to the emulsion layers of said photographic light-sensitive elements, which is not accompanied by the aforesaid drawbacks.

## DESCRIPTION OF THE PREFERRED EMBODIMENTS

According to the present invention, an improved photographic processing for photographic light-sensitive elements is provided in which the photographic light-sensitive elements are processed between a prehardening step and a development step in an aqueous solution containing a resorcinol derivative represented by the general formula



wherein A and B each represent a hydrogen atom, a lower alkyl group, a halogen atom, OR<sub>1</sub> (wherein R<sub>1</sub> represents a lower alkyl group), COR<sub>2</sub> (wherein R<sub>2</sub> represents a hydroxyl group, an alkoxyl group, or NH<sub>2</sub>) or SO<sub>2</sub>R<sub>3</sub> (wherein R<sub>3</sub> represents a hydroxyl group, an alkoxyl group, or NH<sub>2</sub>).

Typical examples of the above resorcinol derivative are resorcin, 4-chlororesorcin, 4,6-dichlororesorcin, 4-methoxresorcin, 4-methylresorcin, and 4-carboxyresorcin.

The concentration of the resorcinol derivative depends upon the concentration of the aldehyde coming from the prehardening processing, but the aldehyde from the prehardening processing can generally be effectively removed at a concentration range of 0.1–100 g./liter of the resorcinol derivative.

The aqueous solution for the antifogging processing may be used at any pH range, but is particularly effective in a neutral state or an acid state. Moreover, the aqueous solution containing the resorcinol derivative may contain pH-controlling agents or buffering agents, such as sodium sulfate, borax, acetic acid, sodium acetate, sodium carbonate, sulfuric acid, and boric acid, as well as other conventional antifogging agents such as an alkali halide.

The photographic emulsion layer to be processed according to the process of this invention contains, as the light sensitive material, conventional silver halides. As the dispersoid for the light-sensitive material, there is generally employed gelatin or a mixture of gelatin and another hydrophilic high molecular weight material. As a support for the photographic emulsion layer, there may be employed a glass plate, a cellulose ester film, a polyester film, a paper, and the like.

The process of this invention is particularly suitable when applied to processing reversal color photographic light-sensitive elements which are desirably processed at a high pH and for a long period of time; and also for processing color photographic printing papers which are preferably quickly processed at a high temperature.

In the practice of the process of this invention, the formation of development fog is low, when compared with a conventional photographic processing. In addition, a reduction in development density does not occur and the coupling property of couplers in color photographic light-sensitive elements is not varied.

The invention will be further explained in detail by the following examples, although the invention shall not be limited to them.

## EXAMPLE 1

A panchromatic gelatino silver iodobromide emulsion layer sufficiently color sensitized (formed on a cellulose acetate film) was exposed by means of a sensitometer and subjected to the following photographic processings at 40°C.

|    | Processing             | Time    |
|----|------------------------|---------|
| 70 | Prehardening           | 35 sec. |
|    | Washing                | 10 sec. |
|    | Antifogging processing | 45 sec. |
|    | Washing                | 20 sec. |
|    | Development            | 50 sec. |
|    | Stopping               | 10 sec. |
| 75 | Fixing                 | 30 sec. |

Washing

90 sec.

The compositions for the processing solutions used in the above processings are as follows:

| Prehardening composition |        |  |
|--------------------------|--------|--|
| Sodium bisulfite         | 1 g.   |  |
| Formalin (37% aq. soln.) | 15 ml. |  |
| Borax                    | 5 g.   |  |
| Sodium sulfate           | 50 g.  |  |
| Potassium bromide        | 2 g.   |  |
| Water to make            | 1 l.   |  |
| Antifogging composition  |        |  |

The resorcinol derivative shown in the following table was added to one liter of an aqueous solution containing 5 g. of glacial acetic acid and 4 g. of sodium acetate.

| Test No.    | Additive                     | Amount |
|-------------|------------------------------|--------|
| 1 (control) | none                         | —      |
| 2           | Resorcin                     | 5 g.   |
| 3           | Resorcin                     | 10 g.  |
| 4           | 4-Chlororesorcin             | 5 g.   |
| 5           | 4-Chlororesorcin             | 10 g.  |
| Developer   |                              |        |
|             | Metol                        | 5 g.   |
|             | Hydroquinone                 | 2 g.   |
|             | Sodium sulfate               | 70 g.  |
|             | Sodium hydroxide             | 1 g.   |
|             | Sodium carbonate monohydrate | 41 g.  |
|             | Potassium bromide            | 2 g.   |
|             | Water to make                | 1 l.   |
|             | Stopping solution            |        |
|             | Glacial acetic acid          | 15 ml. |
|             | Water to make                | 1 l.   |
|             | Fixing solution              |        |
|             | Sodium thiosulfate           | 150 g. |
|             | Sodium sulfite               | 15 g.  |
|             | Water to make                | 1 l.   |

The photographic properties of the test films processed as described above are shown in Table 1.

TABLE 1

| Test No.    | Fog  | Relative sensitivity | Gamma value |
|-------------|------|----------------------|-------------|
| 1 (control) | 0.36 | 2.20                 | 0.32        |
| 2           | 0.27 | 2.30                 | 0.33        |
| 3           | 0.25 | 2.31                 | 0.33        |
| 4           | 0.26 | 2.32                 | 0.35        |
| 5           | 0.23 | 2.32                 | 0.36        |

In Table 1, the relative sensitivity is shown by the logarithmic value of the reciprocal of the exposure amount corresponding to the blackened density of 0.1 over fog.

It is clear from the above results that by the application of the antifogging processing of this invention, the formation of development fog was effectively prevented and the sensitivity, as well as the gamma value, were increased.

Also, by the application of the antifogging bath, the prehardening process can be practically employed to improve the mechanical strength of the emulsion layers. Thus, the light-sensitive elements may be processed at a high temperature without being accompanied by operative troubles.

#### EXAMPLE 2

A panchromatic gelatino silver halide emulsion layer sufficiently color sensitized and formed on a polyester film was exposed by means of a sensitometer through a silver step wedge and then subjected to the following photographic processings at 27°C. (except drying which was conducted at 38°C.).

|    | Processing             | Time     |
|----|------------------------|----------|
| 5  | Prehardening           | 60 sec.  |
|    | Washing                | 30 sec.  |
|    | Antifogging processing | 60 sec.  |
|    | Washing                | 30 sec.  |
| 10 | Primary development    | 210 sec. |
|    | Washing                | 30 sec.  |
|    | Bleaching              | 120 sec. |
|    | Washing                | 30 sec.  |
|    | Cleaning               | 60 sec.  |
|    | Washing                | 30 sec.  |
| 15 | Secondary development  | 120 sec. |
|    | Washing                | 30 sec.  |
|    | Fixing                 | 90 sec.  |
|    | Washing                | 150 sec. |
|    | Drying                 | 180 sec. |

The compositions for the above processings are as follows:

Prehardening composition

Same as in Example 1.

Antifogging composition

The resorcinol derivative shown in the following table was added to one liter of an aqueous solution containing 4 g. of sodium acetate, 5 ml. of glacial acetic acid, and 0.7 g. of potassium bromide.

Primary and secondary developers

0.8 g./liter of potassium thiocyanate was added to the developer in Example 1.

|    | Bleaching solution   |       |  |
|----|----------------------|-------|--|
| 35 | Sulfuric acid        | 5 ml. |  |
|    | Potassium bichromate | 4 g.  |  |
|    | Water to make        | 1 l.  |  |
|    | Cleaning composition |       |  |

|    |                 |       |
|----|-----------------|-------|
| 40 | Sodium sulfite  | 50 g. |
|    | Water to make   | 1 l.  |
|    | Fixing solution |       |

Same as in Example 1.

45 Results of the above processing are shown in the following table.

TABLE 2

| Test No.    | Additives                | Reversal density |
|-------------|--------------------------|------------------|
| 1 (control) | none                     | 1.12             |
| 2           | 4-Chlororesorcinol 2 g.  | 1.43             |
| 3           | 4-Chlororesorcinol 5 g.  | 1.46             |
| 4           | 4-Chlororesorcinol 10 g. | 1.48             |

55 It is clear from the above results that the reversal density was increased by using the antifogging bath according to the process of this invention; hence, better photographic properties were obtained in the photographic film thus processed in spite of the application of the prehardening processing.

60 Moreover, during the processing of this invention, the surface of the emulsion layer was less damaged mechanically, and the drying load could be reduced.

#### EXAMPLE 3

A multiple layer photographic color film prepared by applying to a cellulose acetate film a gelatino silver iodobromide emulsion having a red sensitivity, a gelatino silver iodo-bromide emulsion having a green sensitivity, a yellow filter layer containing fine colloidal silver particles and having a blue-absorptive property, and a gelatino silver iodobromide emulsion having a blue sensitivity (in this order) was exposed through a silver step wedge by means of a sensitometer and then subjected to the following photographic processings at 24°C.

| 75 | Processing | Time |
|----|------------|------|
|----|------------|------|

|                        |        |
|------------------------|--------|
| Prehardening           | 1 min. |
| Washing                | 1 min. |
| Antifogging processing | 1 min. |
| Washing                | 1 min. |
| Primary development    | 5 min. |
| Washing                | 2 min. |

Reversal exposure at 200 CMS (red light) from the back side of the film.

|                        |        |
|------------------------|--------|
| Cyan color development | 5 min. |
| Washing                | 2 min. |

Reversal exposure (blue light) at 200 CMS from the emulsion side of the film.

|                          |        |
|--------------------------|--------|
| Yellow color development | 5 min. |
| Washing                  | 1 min. |
| Secondary development    | 1 min. |
| Washing                  | 1 min. |

Reversal exposure (white light) at 2000 CMS. from the opposite sides of the film.

|                           |        |
|---------------------------|--------|
| Magenta color development | 5 min. |
| Washing                   | 5 min. |
| Bleaching                 | 2 min. |
| Washing                   | 1 min. |
| Fixing                    | 2 min. |
| Washing                   | 2 min. |

The compositions for the above processings were as follows:

Prehardening composition  
Same as in Example 1.

Antifogging composition

The resorcinol derivative shown in the following table was added to one liter of an aqueous solution containing 8 g. of boric acid, 0.3 ml. of sulfuric acid, and 0.8 g. of potassium bromide to provide the antifogging bath.

|                                             |         |
|---------------------------------------------|---------|
| 1-Phenyl-3-(m-nitrobenzoylamo)-5-pyrazolone | 1.4 g.  |
| Sodium hydroxide                            | 2.0 g.  |
| n-Butylamine                                | 5.0 ml. |
| Water to make                               | 1 l.    |
| Bleaching composition                       |         |

|                        |          |
|------------------------|----------|
| Potassium ferricyanide | 100.0 g. |
| Potassium bromide      | 20.0 g.  |
| Borax                  | 2.0 g.   |
| Boric acid             | 1.0 g.   |
| Water to make          | 1 l.     |
| Fixing composition     |          |

|                    |        |
|--------------------|--------|
| Sodium thiosulfate | 150 g. |
| Sodium sulfite     | 10 g.  |
| Water to make      | 1 l.   |

The results are shown in the following table.

TABLE 3

| Test No.    | Red density | Green density | Blue density |
|-------------|-------------|---------------|--------------|
| 1 (control) | 3.05        | 2.95          | 2.90         |
| 2           | 3.39        | 3.31          | 3.38         |
| 3           |             | 3.40          | 3.40         |
| 4           |             | 3.40          | 3.45         |
| 5           |             | 3.44          | 3.48         |

It is clear from the above table that the coupling density was remarkably increased by employing the antifogging processing according to the process of this invention, and no harmful influence on the photographic properties were observed, that is, contamination and sensitivity reduction were not observed.

## EXAMPLE 4

A commercially available photographic color printing paper was exposed by means of a sensitometer and processed as follows at 20° C.

|                                                            |         |
|------------------------------------------------------------|---------|
| Sodium bisulfite                                           | 4.0 g.  |
| Water to make                                              | 1 l.    |
| Buffering solution                                         |         |
| Tartaric acid                                              | 10.0 g. |
| Borax                                                      | 25.0 g. |
| Water to make                                              | 1 l.    |
| Stabilization composition                                  |         |
| Whitening agent (Tinopol; trade name, made by Geigy A. G.) | 4.0 g.  |
| Sodium dihydrogen phosphate                                | 4.0 g.  |
| Disodium hydrogen phosphate                                | 2.0 g.  |
| Tetrasodium salt of ethylene-diamine-tetraacetic acid      | 1.0 g.  |
| Water to make                                              | 1 l.    |

By the practice of Processing I, good photographic qualities in the photographic print were obtained, but it was accompanied by one fault, i.e., the printing paper had to be processed for a longer period of time (as shown above).

Therefore, to shorten the processing time, the printing paper was processed at 35° C. (Processing II). In this case, a so-called "reticulation" formed on the emulsion layer, which reduced the commercial value of the printing paper.

A hardening procedure was then conducted before the 25 color development (Processing II). That is, instead of the hardening procedure, in Processing I, the printing paper was processed for 60 seconds before color development in a hardening bath having the following composition:

| Hardening composition        |        |
|------------------------------|--------|
| Formalin (37% aq. soln.)     | 20 ml. |
| 2,5-Dimethoxytetrahydrofuran | 4 ml.  |
| Sulfuric Acid                | 2 ml.  |
| Sodium sulfate               | 100 g. |
| Potassium bromide            | 2 g.   |
| Borax                        | 5 g.   |
| Water to make                | 1 l.   |

By the practice of Processing III, intense development fogs formed, although the mechanical strength of the emulsion layer was improved. Hence, the commercial value of the printing paper was nonetheless lost (as in Processing II).

Accordingly, Processing IV of this invention employing the antifogging processing was conducted, and by this procedure better photographic qualities as in Processing I were obtained. Moreover, the printing paper could be processed in a short period of time, as shown below, while maintaining sufficient mechanical strength of the light-sensitive emulsion layer. This processing was conducted at 38° C.

| Processing IV          | Time     |
|------------------------|----------|
| Hardening              | 60 sec.  |
| Washing                | 30 sec.  |
| Antifogging processing | 60 sec.  |
| Washing                | 30 sec.  |
| Color development      | 100 sec. |
| Washing                | 30 sec.  |
| Bleach-fixing          | 140 sec. |
| Washing                | 30 sec.  |
| Buffering              | 40 sec.  |
| Washing                | 30 sec.  |
| Stabilization          | 40 sec.  |
| Drying (at 50° C.)     |          |

The antifogging bath used in the process was an aqueous solution containing 10 g./liter of 4-chlororesorcin and 0.5 g./liter of potassium bromide. The hardening bath was the same as in Processing III.

The fog densities of the printing papers processed by Processings I, II, III, and IV are shown in the following table.

| Processing | Fog Density |               |              |
|------------|-------------|---------------|--------------|
|            | Red Density | Green Density | Blue Density |
| I          | 0.08        | 0.08          | 0.11         |
| II         | —           | —             | —            |
| III        | 0.35        | 0.20          | 0.45         |
| IV         | 0.09        | 0.09          | 0.11         |

TABLE 4

EXAMPLE 5

10 A gelatino silver halide emulsion layer having a red sensitivity formed on a cellulose acetate film was exposed through a silver step wedge by means of a sensitometer and subjected to the following reversal color processing, at 24° C.

| Processing             | Time     |
|------------------------|----------|
| Prehardening           | 60 sec.  |
| Washing                | 60 sec.  |
| Antifogging processing | 60 sec.  |
| Washing                | 60 sec.  |
| Primary development    | 210 sec. |
| Washing                | 60 sec.  |

Reversal exposure at 200 MS. under white light.

|    |                        |          |
|----|------------------------|----------|
| 30 | Cyan color development | 210 sec. |
|    | Washing                | 60 sec.  |
|    | Bleaching              | 60 sec.  |
|    | Washing                | 60 sec.  |
|    | Fixing                 | 60 sec.  |
|    | Washing                | 60 sec.  |

The compositions of the prehardening bath and the antifogging bath used were the same as in Example 1, the other 35 compositions being the same as in Example 3. The results are shown in the following table.

TABLE 5

| Test No.    | Additive             | Amount | Reversal Density |
|-------------|----------------------|--------|------------------|
|             |                      |        | (red density)    |
| 1 (control) | none                 |        | 0.55             |
| 2           | Resorcin             | 5 g.   | 1.01             |
| 3           | 4-Chlororesorcin     | 5 g.   | 1.12             |
| 4           | 4,6-Dichlororesorcin | 5 g.   | 1.10             |
| 5           | 4-Methoxyresorcin    | 5 g.   | 1.05             |
| 6           | 4-Methylresorcin     | 5 g.   | 1.04             |

It is clear from the above results that by the use of the antifogging bath, coupling density was remarkably increased.

A reversal magenta color development was conducted basically as in Example 5. Specifically, the procedure of Example 5 was repeated employing the magenta color developer shown in Example 3 instead of the cyan color developer of Example 5, and an antifogging composition as shown in the following table was instead employed. The antifogging bath was in aqueous solution containing 50 g./liter of sodium sulfate, 5.0 g./liter of sodium bisulfite, 1.0 g. of boric acid, and 0.5 g./liter of potassium bromide, together with the following resorcin 60 derivative.

| Test No.    | Additive             | Amount (g./l.) |
|-------------|----------------------|----------------|
| 1 (control) | none                 |                |
| 2           | Resorcin             | 5              |
| 3           | 4-Chlororesorcin     | 5              |
| 4           | 4,6-Dichlororesorcin | 5              |
| 5           | 4-Methoxyresorcin    | 5              |
| 6           | 4-Methylresorcin     | 5.             |

Results are shown in the following table.

TABLE 6

| Test No.    | Reversal dens | ity (green density) |
|-------------|---------------|---------------------|
| 1 (control) | 1.50          |                     |
| 2           | 2.32          |                     |
| 3           | 2.42          |                     |
| 4           | 2.40          |                     |

|   |      |
|---|------|
| 5 | 2.35 |
| 6 | 2.37 |

As shown in the above table, the coupling density was markedly increased by employing the antifogging processing of this invention.

What is claimed is:

1. In a photographic processing sequence for gelatin-containing photographic silver halide light-sensitive elements including immersing said light-sensitive elements in a prehardening bath prior to development, said prehardening bath containing an aldehyde hardening agent capable of hardening said gelatin, the improvement which comprises processing the light-sensitive elements between the prehardening bath and the development in an aqueous solution containing 0.1 to 100 g./liter of the aqueous solution of a resorcinol derivative represented by the following general formula



10 wherein A and B each represents a member selected from the group consisting of a hydrogen atom, a lower alkyl group, a halogen atom, OR<sub>1</sub>, wherein R<sub>1</sub> is a lower alkyl group, COR<sub>2</sub>, wherein R<sub>2</sub> is a member selected from the group consisting of

5 a hydroxyl group, an alkoxy group, and NH<sub>2</sub>, and SO<sub>2</sub>R<sub>3</sub>, wherein R<sub>3</sub> is a member selected from the group consisting of

a hydroxyl group, an alkoxy group, and NH<sub>2</sub>.

2. The photographic processing as claimed in claim 1 wherein said resorcinol derivative is selected from the group consisting of resorcin, 4-chlororesorcin, 4,6-dichlororesorcin, 4-methoxyresorcin, 4-methylresorcin, and 4-carboxyresorcin.

3. A photographic processing as claimed in claim 1 wherein said photographic silver halide light-sensitive element comprises a silver halide and a mixture of gelatin with another hydrophilic high molecular weight material.

4. The photographic processing as claimed in claim 1 wherein said aldehyde is selected from the group consisting of formaldehyde, glyoxal, succinaldehyde and glutaraldehyde.

20

\* \* \* \* \*

25

30

35

40

45

50

55

60

65

70

75